

## UNITED STATES PATENT OFFICE.

NOAK VICTOR HYBINETTE, OF WILMINGTON, DELAWARE.

NICKEL ANODE AND PROCESS FOR MANUFACTURING THE SAME.

No Drawing.

Application filed June 3, 1922. Serial No. 565,753.

*To all whom it may concern:*

Be it known that I, NOAK VICTOR HYBINETTE, a citizen of the United States, residing at Wilmington, in the county of New Castle, State of Delaware, have invented certain new and useful Improvements in Nickel Anodes and Processes for Manufacturing the Same; and I do hereby declare the following to be a full, clear, and exact description of the invention, such as will enable others skilled in the art to which it appertains to make and use the same.

This invention relates to improved nickel anodes and to a process of producing such anodes substantially free from impurities which interfere with the production of malleable nickel by the electrolytic method.

For certain purposes, such as the production of malleable electrolytic nickel, it is necessary that the anode should be of extreme purity. These should particularly be no carbon, silicon or chromium, and it is desirable that the iron contents should be lower than they usually are in the commercial nickel.

My anode consists of a casting produced by oxidizing ordinary commercial nickel in a certain way so that a solid plate can be produced therefrom which is free from lead, carbon and silicon, and can be made to contain less than 0.25 per cent and preferably less than 0.15 to 0.1 per cent of iron. A particularly desirable characteristic of the anode is its oxygen content amounting to at least one-tenth of one per cent. The presence of oxide increases the solubility of the anode in the electrolyte.

To produce the anode ordinary nickel is smelted in a reverberatory furnace and oxidized either by the addition of nickel oxide or by oxidizing furnace gases during the smelting down period, or by blowing on it with compressed air after the metal is all smelted. By this smelting down with or without any slagging material under oxidizing conditions, I am able to remove such impurities as lead and possibly some part of the sulphur contained in the original metal.

The next step in the process has the object of removing iron. Ordinarily one would think that silicate of nickel would enter into a reaction with oxide of iron dissolved in the metal so that silicate of iron will enter the slag and a corresponding quantity of nickel take its place in the metal. Inas-

much as nickel silicate and nickel oxide are infusible at ordinary furnace temperatures, this reaction does not take place and I find it necessary to produce a slag which will hold the nickel silicate in solution. I have also found that it is necessary to supply such slag in considerable quantity so that the silicates of nickel and iron will be very diluted. Supposing, therefore, that the commercial nickel which is used as raw material contains 1 per cent of iron and it is required to bring the iron contents down to 0.25 per cent, I find that I obtain the best results by calculating that I have to produce a slag containing the quantity of iron to be removed to the extent of 3 per cent. The slag has also at the same time to contain about four times as much nickel, say 10—12 per cent. The remainder of the slag has to be made up of silicates of lime, magnesia, and alumina in varying quantities. In practice I make use of ordinary gravel or sand with an addition of lime so as to make a slag consisting mainly of silicate of lime but containing enough other silicates to make a perfectly fused slag at the temperature of the furnace, say about 1550° C. It is not necessary that the slag should be particularly basic or particularly acid, and for the sake of protecting the furnace walls I prefer to have a nearly neutral slag. In round figures I add 250 pounds of a mixed silicate of lime, magnesia and alumina for 1000 pounds nickel. There is a certain improvement in the degree to which the reaction works if the slag is made to contain fluxes such as soda, borax, fluorspar, etc., but it is not necessary to use them. When this slag is thrown on the metal and fused, I find that a large quantity of the oxides that were before dissolved in the metal are absorbed by the slag, and that in this particular case nickel and iron enter the slag in the proportion of about four parts of nickel to one part of iron. If the preliminary oxidizing has not been sufficient, I add nickel oxide or I blow on the bath with a powerful blast of air that will penetrate the slag and oxidize the metal beneath. In this way I oxidize until the desired amount of iron has been removed from the metal. The slag is then poured off and if necessary a second slag may be put on and the procedure repeated, but for all practical purposes I find that one slagging operation is sufficient.

The slag has a certain value on account of its high nickel contents and is utilized as raw material for nickel production in any well known way.

5. The process may be varied by smelting the slag with the metal and allowing the metal to remain uncovered in the furnace for some time after the iron slag is removed, but I prefer to do the smelting down without slag. It is evident that some volatile metals such as lead are more completely removed by such exposure of the molten metal to the furnace gases.

10. The metal from which now all the impurities have been removed is preferably covered with a neutral slag so as to protect it from the furnace gases and it contains about one-half to one per cent of nickel oxide or a quantity of oxygen corresponding to that 15 amount of nickel oxide and preferably not less than 0.1 per cent. Ordinarily oxidized nickel is supposed to be unsuitable for any practical use because when pouring it into molds it gives off gases and segregates 20 nickel oxide so as to produce a spongy metal of insufficient strength and of varying composition. But I find that if I regulate the oxygen contents within the limits now 25 mentioned, solid metal suitable for anodes 30 is obtained.

Various changes may be made in the details of the operation as hereinbefore described without departing from the invention or sacrificing any of the advantages 35 thereof.

I claim:—

1. A nickel anode containing at least one-tenth of one per cent of oxygen.
2. A nickel anode containing oxygen.
3. A cast nickel anode containing oxygen and substantially free from carbon and silicon.
4. A cast nickel anode containing oxygen

and substantially free from carbon, silicon and chromium.

5. A cast nickel anode containing oxygen and substantially free from carbon, silicon, chromium and lead.

6. A cast nickel anode containing oxygen and less than 0.15 per cent of iron.

7. A nickel anode containing oxygen and less than 0.15 per cent of iron.

8. A process of producing the nickel anode described in claim 1, consisting in smelting ordinary commercial nickel with the addition of an oxidizing agent and a slag capable of dissolving metallic oxides, thereby producing purified and oxidized metal suitable to be cast into an anode.

9. A process for producing pure nickel 60 anodes which consists in oxidizing the impurities in the nickel in the presence of a quantity of slag at least substantially equal to ten times the weight of the iron to be removed from the nickel.

10. A process for producing pure nickel 65 anodes which consists in oxidizing the impurities in the nickel in the presence of a quantity of slag varying from ten to thirty times the weight of the iron to be removed 70 from the nickel.

11. A process of producing nickel anodes substantially free from lead and iron, which comprises subjecting a molten bath of nickel to an oxidizing agent and continuing the 75 oxidation in the presence of a slag capable of dissolving the iron.

12. The process of producing nickel anodes substantially free from lead and iron, which comprises subjecting a molten bath of 80 nickel to an oxidizing agent in the presence of a slag capable of dissolving the iron, and exposing the molten metal during a period in the oxidizing operation.

In testimony whereof I affix my signature.

NOAK VICTOR HYBINETTE.